

Patented Aug. 16, 1927.

1,638,855

# UNITED STATES PATENT OFFICE.

LOUIS JORDAN AND GEORGE WILLARD QUICK, OF WASHINGTON, DISTRICT OF COLUMBIA, ASSIGNORS TO THE UNITED STATES OF AMERICA, REPRESENTED BY THE SECRETARY OF COMMERCE.

## ALLOY.

No Drawing.

Application filed December 27, 1926. Serial No. 157,433.

(GRANTED UNDER THE ACT OF MARCH 3, 1883; 22 STAT. L. 625.)

This application having been made pursuant to the provisions of the act of March 3, 1883 (ch. 143, 22 Stat. L., 625), we hereby declare that this invention may be used pursuant to the terms of said act reading as follows: "Provided, That the applicant in his application shall state that the invention described therein, if patented, may be used by the Government, or any of its officers or employees in prosecution of work for the Government, or by any other person in the United States, without the payment to him of any royalty thereon, which stipulation shall be included in the patent."

15 Our invention relates to alloys of iron, carbon and vanadium, and has for its object to produce such alloys having great hardness combined with malleability and toughness, and which can be further hardened by suitable heat treatment without becoming brittle, and still further hardened by cold working after hardening by heat treatment.

20 A further object of our invention is to provide an alloy which is suitable for the preparation of balls for use in measuring the Brinell hardness of extremely hard steels, or for other uses.

Iron-carbon-vanadium alloys pursuant to our invention contain much larger proportions of carbon than alloys ordinarily designated as steels, and also contain much larger proportions of vanadium than what are known as vanadium steels. Pursuant to our invention, our alloys may contain from approximately 2 to 4 percent carbon, and from approximately 10 to 15 percent vanadium, together with comparatively small amounts of the impurities or deoxidizers usually present in commercial ferrous alloys, such as manganese, sulphur, silicon and phosphorus.

As an illustrative example of our invention, we give the following:

|                     | Per cent. |
|---------------------|-----------|
| 45 Carbon           | 2.93      |
| Vanadium            | 13.5      |
| Manganese           | .10       |
| Sulphur             | .016      |
| Silicon             | 1.55      |
| 50 Iron, balance to | 100       |

The carbon and vanadium to the proper

amounts are incorporated with the iron in the usual way of making such alloys.

It will be understood that the proportions above given are not to be taken as restrictive or limiting, but as only one example. The proportions of the vanadium and carbon may be varied within the approximate limits above stated.

We have found that alloys of the above compositions may be given greatly increased hardness by suitable heat treatment. For example, quenching such alloy from temperatures between 850 to 925° C. and tempering at 100° C. produces a metal of greater hardness than ordinary high carbon quenched steels. Still further hardness may be produced in such quenched and tempered alloys by cold working, as for example, by cold working of quenched and tempered balls of these alloys by the well known method of work hardening balls, described by Hultgren (Jour. Iron and Steel Inst., 1924, No. II, page 183).

Alloys produced in accordance with our invention possess also toughness and malleability, and do not become brittle or short by the further hardening treatments described.

What we claim is—

1. An iron alloy containing from approximately 2 to approximately 4 per cent carbon, and from approximately 10 to approximately 15 per cent vanadium.

2. An iron alloy containing substantially 3 per cent carbon and substantially 13.5 per cent vanadium.

3. An iron vanadium-carbon alloy containing from approximately 2 to approximately 4 per cent carbon, and from approximately 10 to approximately 15 per cent vanadium and having the characteristics of great hardness combined with toughness and malleability and which is susceptible of further hardening without becoming brittle by heating and quenching and which may be still further hardened by cold working after such heat treatment.

LOUIS JORDAN.  
GEORGE WILLARD QUICK.